# EUROPEAN PATENT SPECIFICATION

(11) **EP 1 640 466 B1**
(45) Date of publication and mention of the grant of the patent: **05.08.2009**
(21) Application number: 05020951.9
(22) Date of filing: 26.09.2005
(51) Int. Cl.: C22C 23/04, C22F 1/06

(54) **Magnesium alloy and production process thereof**
Magnesiumlegierung und Herstellungsverfahren
Alliage de magnésium et procédé de fabrication

(30) Priority: 28.09.2004 JP 2004280878
(43) Date of publication of application: 29.03.2006
(73) Proprietor: Kumamoto University, Kumamoto-shi Kumamoto 860-8555 (JP); Honda Motor Co., Ltd., Minato-ku Tokyo 107-8556 (JP); Fuji Light Metal Co., Ltd., Tamana-gun Kumamoto 869-0192 (JP); THE JAPAN STEEL WORKS, LTD., Tokyo 100-8456 (JP)
(72) Inventor: Ienaga, Yuuichi K.K. Honda Gijutsu Kenkyusho, Wako-shi Saitama 351-0193 (JP); Kozono, Ei Fuji Light Metal Co., Ltd., Tamana-gun Kumamoto 869-0192 (JP); Kawamura, Yoshihito, Kumamoto-shi Kumamoto 861-8028 (JP); Yamaguchi, Takeshi The Japan Steel Works, Ltd., Hiroshima-shi Hiroshima 736-8602 (JP)
(74) Representative: Böhm, Brigitte

(56) References cited:
- EP-A- 0 575 796
- US-A1- 2003 029 526
- PATENT ABSTRACTS OF JAPAN vol. 2003, no. 01, 14 January 2003 (2003-01-14) -& JP 2002 256370 A (JAPAN SCIENCE & TECHNOLOGY CORP; MATSUSHITA MITSUHIDE), 11 September 2002 (2002-09-11)
- DATABASE INSPEC [Online] THE INSTITUTION OF ELECTRICAL ENGINEERS, STEVENAGE, GB; January 1989 (1989-01), MURATOVA E V ET AL: "Phase equilibria in the Mg-Y-La-Zn system at temperatures below the solidus" XP002349969 Database accession no. 3606647 -& Inorganic Materials USA, vol. 25, no. 1, January 1989 (1989-01), pages 50-54, XP008054202 ISSN: 0020-1685
- DATABASE INSPEC [Online] THE INSTITUTION OF ELECTRICAL ENGINEERS, STEVENAGE, GB; 15 June 1997 (1997-06-15), SUGAMATA M ET AL: "Structures and mechanical properties of rapidly solidified Mg-Y based alloys" XP002349970 Database accession no. 5694945 -& NINTH INTERNATIONAL CONFERENCE ON RAPIDLY QUENCHED AND METASTABLE MATERIALS 25-30 AUG. 1996 BRATISLAVA, SLOVAKIA, vol. A226-228, 1997, pages 861-866, XP008054234 Materials Science & Engineering A (Structural Materials: Properties, Microstructure and Processing) Elsevier Switzerland ISSN: 0921-5093
- DATABASE INSPEC [Online] THE INSTITUTION OF ELECTRICAL ENGINEERS, STEVENAGE, GB; April 2003 (2003-04), WATANABE H ET AL: "Mechanical properties of Mg-Y-Zn alloy processed by equal-channel-angular extrusion" XP002349971 Database accession no. 7729726 -& Materials Transactions Japan Inst. Metals Japan, vol. 44, no. 4, 2003, pages 463-467, XP008054213 ISSN: 1345-9678
- DATABASE INSPEC [Online] THE INSTITUTION OF ELECTRICAL ENGINEERS, STEVENAGE, GB; 1 May 2000 (2000-05-01), LUO Z P ET AL: "High-resolution electron microscopy on the X-Mg12ZnY phase in a high strength Mg-Zn-Zr-Y magnesium alloy" XP002350242 Database accession no. 6606719 -& Journal of Materials Science Letters Kluwer Academic Publishers USA, vol. 19, no. 9, 2000, pages 813-815, XP008054200 ISSN: 0261-8028
- PATENT ABSTRACTS OF JAPAN vol. 2003, no. 12, 5 December 2003 (2003-12-05) -& JP 2004 099941 A (JAPAN SCIENCE & TECHNOLOGY CORP), 2 April 2004 (2004-04-02)

## Description

The present invention relates to a magnesium alloy having both high strength and high ductility; and a production process thereof.

### Description of the Related Art

Since magnesium is lighter in weight than iron or aluminum, its use as a light-weight substitute for members made of an iron steel material or aluminum alloy material is under investigation. Ordinary magnesium alloys have, however, lower strength than the other metal structure materials such as iron steel, aluminum alloy and titanium alloy. An AZ91 material for die casting, which is said to have relatively high strength, has strength as low as 160 MPa. In addition, industrial parts are required to have, at a moving part thereof, a percent elongation of at least 4 to 5%, but ordinary magnesium alloys do not have sufficient ductility. Even the above-described AZ91 material has a percent elongation of only about 3%.

A variety of magnesium alloys equipped with both high strength and high ductility have so far been proposed.

For example, known is a magnesium alloy having a composition represented by the formula: Mg_{100-a-b-c}CaₐZn_{b}X_{c} (wherein, X represents one or more than one elements selected from the group consisting of Y, Ce, La, Nd, Pr, Sm and Mm (misch metal); and 0.5 ≤ a ≤ 5 atomic %, 0 < b ≤ 5 atomic %, and 0 < c ≤ 3 atomic % with the proviso that 1 ≤ a+b+c ≤ 11 atomic %), and having a structure in which one or more of Mg-Ca, Mg-Zn and Mg-X intermetallic compounds have been finely dispersed in a Mg mother phase composed of a fine crystalline material. The above-described magnesium alloy having intermetallic compound(s) can be obtained as a high strength magnesium alloy in the powder form by rapid solidification of a molten alloy having the above-described composition by atomization or the like method. It can be molded or formed into even complex shaped products by hot plastic processing (refer to Japanese Patent Laid-Open No. 41065/1997).

Also known is a magnesium alloy having a composition represented by the formula: Mg₁₀₀-ₐ-_{b}LnₐM_{b} (wherein, M is one or more elements selected from Al and Zn; Ln is one or more elements selected from Y, Ce, La, Nd, Pr, Pm, Sm, Eu, Gd, Tb, Dy, Ho, Er, Tm, Yb, Lu and Mm (misch metal), or a mixture of rare earth elements; and 0.5 ≤a ≤ 5 atomic %, and 0.2 ≤ b ≤ 4 atomic %, with the proviso that 1.5 ≤ a+b ≤ 7 atomic %); having a crystal grain size less than 2,000 nm; and having a long period hexagonal structure in a part or whole region of the crystals. The above-described magnesium alloy having a long period hexagonal structure can be prepared as a high strength and high ductility magnesium alloy in the powder form by rapid solidification of a molten alloy having the above-described composition by atomization or the like method. By subjecting the resulting powder to plastic processing at an extrusion ratio of from 3 to 20, extrusion goods made of the magnesium alloy can be obtained (refer to Japanese Patent Laid-Open No. 2002-256370).

The above-described magnesium alloys however have a drawback: a yield at the time of rapid solidification of the molten alloy is low, which inevitably leads to a cost rise when the powder obtained by rapid solidification is molded or formed.

The above-described magnesium alloys each has a percent elongation not greater than 5%, which is almost a limit value when they are used for moving portions of industrial parts. Thus, they do not have sufficient ductility. The industrial parts using the above-described magnesium alloys therefore have a drawback: design freedom is greatly limited and they are not suited for practical use.

The magnesium alloy having a long period hexagonal structure, on the other hand, is said so that it could be formed into a molded product by casting using a copper mold with a large cooling rate. When the copper mold is used, however, molded products thus obtained must be relatively small in order to raise its cooling rate. Thus, this magnesium alloy has a drawback that any size of a molded product cannot be produced freely.

### SUMMARY OF THE INVENTION

An object of the present invention is to overcome the above-described drawbacks and provide a magnesium alloy which is inexpensive, has a good yield, can be molded or formed into any size, and has both high strength and high ductility; and a production method of the magnesium alloy.

With a view to attaining the above-described object, the magnesium alloy of the present invention comprises from 1 to 4 atomic % of Zn and from 1 to 4.5 atomic % of Y and optionally from 0.1 to 0.5 atomic % of Zr , each based on the total amount and as a remaining portion Mg and inevitable impurities, at a Zn/Y composition ratio falling within a range of from 0.6 to 1.3, and further comprises Mg₃Y₂Zn₃ which is an intermetallic compound and Mg₁₂YZn having a long period structure.

Since the magnesium alloy according to the present invention has, as well as the above-described composition, both the intermetallic compound Mg₃Y₂Zn₃ and Mg₁₂YZn having a long period structure, it is able to have both high strength and high ductility. Either one of or both of strength and ductility become insufficient when the content of Zn is less than 1 atomic % or exceeds 4 atomic % and that of Y is less than 1 atomic % or exceeds 4.5 atomic %, based on the total amount of the magnesium alloy.

Even if Zn and Y both satisfy the above-described ranges based on the total amount of the magnesium alloy, either one or both of strength and ductility becomes insufficient when the magnesium alloy is free of either one or both of the intermetallic compound Mg₃Y₂Zn₃ and Mg₁₂YZn having a long period structure.

In addition, the magnesium alloy of the present invention is required to satisfy the Zn/Y composition ratio which falls within a range of from 0.6 to 1.3 in order to incorporate both the intermetallic compound Mg₃Y₂Zn₃ and Mg₁₂YZn having a long period structure in the alloy without failure. When the Zn/Y composition ratio is less than 0.6 or exceeds 1.3, the magnesium alloy does not always contain either one or both of the intermetallic compound Mg₃Y₂Zn₃ and Mg₁₂YZn having a long period structure.

It is known in a rapidly solidified Mg-Zn-Y alloy that an alloy of MgZₙYₓ (X=2 to 4) in which the concentration of Y > the concentration of Zn has an increased long period structure as the concentration of Y becomes greater; in the case of an alloy of MgZnₓY (X=2 to 4) in which the concentration of Zn > the concentration of Y, heat treatment of it causes precipitation of the intermetallic compound Mg₃Y₂Zn₃; and an alloy of MgZnₓYₓ (X=1 to 4) in which the concentration of Y = the concentration of Zn, that is, an equiatomic alloy is heat treated to generate the long period structure (refer to: Masayuki Nagano, Minoru Nishida, and Yoshihito Kawamura, "Influences of concentrations of Zn and Y and heat treatment on the structure formation of rapidly solidified Mg-Zn-Y alloy", Collected Abstracts of the 2003 meeting of the Japan Institute of Metals, The Japan Institute of Metals, p187).

According to the investigation by the present inventors, however, no intermetallic compound Mg₃Y₂Zn₃ exists in each of the alloy in which the concentration of Y > the concentration of Zn and the equiatomic alloy in which the concentration of Y = the concentration of Zn, while no long period structure exists in the alloy in which the concentration of Zn > the concentration of Y. Accordingly, the long period structure and intermetallic compound Mg₃Y₂Zn₃ do not exist simultaneously in the rapidly solidified Mg-Zn-Y alloy.

The magnesium alloy of the present invention preferably contains from 2 to 3.5 atomic % of Zn and from 2 to 4.5 atomic % of Y and optionally from 0.1 to 0.5 atomic % of Zr, each based on the total amount and as a remaining portion Mg and inevitable impurities , at a Zn/Y composition ratio falling within a range of from 0.8 to 1.2, in order to have both higher strength and higher ductility.

Incorporation of Zr in the magnesium alloy of the present invention within the above-descried range enables to impart a miniaturized alloy structure to the magnesium alloy. Miniaturization effect of the alloy structure cannot be attained when the content of Zr is less than 0.1 atomic % based on the total alloy amount. On the other hand, when the content of Zr exceeds 0.5 atomic % based on the total alloy amount, formation of the intermetallic compound Mg₃Y₂Zn₃ is sometimes disturbed.

The magnesium alloy of the present invention is able to have higher strength by the addition, to the above-described composition, of a small amount of at least one element selected from the group consisting of La, Ce, Nd, Sm and Yb. Moreover, the magnesium alloy of the present invention can be obtained as a composite by adding a reinforcing material such as fibers and particles.

The magnesium alloy of the present invention can be produced by a process comprising casting an Mg alloy containing from 1 to 4 atomic % of Zn and from 1 to 4.5 atomic % of Y and optionally from 0.1 to 0.5 atomic % of Zr, each based on the total amount and as a remaining portion Mg and inevitable impurities, at a Zn/Y composition ratio falling within a range of from 0.6 to 1.3; using a cooling rate of 10 K/sec or less and a metal mould, graphite mould or sand mould and plastic processing of the cast product obtained in the above-described step into an alloy structure containing an intermetallic compound Mg₃Y₂Zn₃ and Mg₁₂YZn having a long period structure.

### DESCRIPTION OF THE PREFERRED EMBODIMENTS

Embodiments of the present invention will hereinafter be described more specifically.

In this Embodiment, a material containing from 1 to 4 atomic % of Zn and from 1 to 4.5 atomic % of Y and optionally from 0.1 to 0.5 atomic % of Zr, each based on the total alloy amount, at a Zn/Y composition ratio falling within a range of from 0.6 to 1.3, and as a remaining portion, Mg and inevitable impurities is charged in a carbon crucible. In an argon atmosphere, the material is melted in a high-frequency melting furnace, for example, at 700°C to yield a molten alloy.

The molten alloy is poured into a mold, followed by casting. A cooling rate during the casting is preferably 10 K/sec or less. This cooling rate is much lower than that of atomization method or twin-roll method employed for rapid solidification, that is, 10⁴ K/sec or greater. It is also much lower than that of roll casting method or quenched copper mold method, that is, 10³ to 10² K/sec. In this Embodiment, ordinarily employed molds such as metal mold, graphite mold and sand mold can be used for casting and a copper mold or water-cooled copper mold is not necessary, which leads to a reduction in the production cost.

The cast product thus obtained is subjected to plastic processing, whereby a molded or formed product can be obtained. The molded or formed product is a magnesium alloy containing from 1 to 4 atomic % of Zn and from 1 to 4.5% of Y and optionally from 0.1 to 0.5 atomic % of Zr, based on the total alloy amount, at a Zn/Y composition ratio falling within a range of from 0.6 to 1.3 and as a remaining portion Mg and inevitable impurities. It contains both an intermetallic compound Mg₃Y₂Zn₃ and Mg₁₂YZn having a long period structure. As a result, the molded or formed product is able to have both high strength and high ductility.

Examples, Comparative examples and Referential Examples of the present invention will next be described.

### [Examples]

In Examples, materials containing, based on the total alloy amount, from 1 to 4 atomic % of Zn and from 1 to 4.5 atomic % of Y at a Zn/Y composition ratio falling within a range of from 0.6 to 1.3 and optionally from 0.1 to 0.5 atomic % of Zr, and, as a remaining portion, Mg and inevitable impurities, which materials were however different from each other with their amounts of Zn, Y and Zr varied within the above-described ranges were charged in a carbon crucible. In an argon atmosphere, the materials were melted in a high-frequency melting furnace, for example, at 700°C. The molten alloys thus obtained were poured into metal molds, followed by casting at a cooling rate not greater than 10K/sec, whereby rod materials were obtained. The rod materials were heated to a temperature range of from 350 to 450°C in an electric furnace, and then extruded at an extrusion ratio of 10, whereby extrusion goods were obtained.

The metal structure of each of the resulting extrusion goods was identified by X-ray diffraction and transmission electron microscope, whereby the presence or absence of an intermetallic compound Mg₃Y₂Zn₃ and Mg₁₂YZn having a long period structure was confirmed. Test pieces were cut from the extrusion goods. Their 0.2% proof stress, tensile strength and elongation were measured by conducting a tensile test on them at normal temperature. The results are shown in Table 1.

### [Comparative Examples]

In Comparative Examples, in a similar manner to that employed for the above-described Examples except that materials containing, each based on the total alloy amount, from 0.5 to 5 atomic % of Zn and from 0.5 to 5 atomic % of Y and containing, as a remaining portion, Mg and inevitable impurities, which materials were however different from each other with their amounts of Zn and Y varied within the above-described ranges were used, rod materials were obtained. The rod materials were extruded as in the above-described Examples, whereby extrusion goods were obtained.

The metal structure of each of the resulting extrusion goods was identified by X-ray diffraction and transmission electron microscope, whereby the presence or absence of an intermetallic compound Mg₃Y₂Zn₃ and Mg₁₂YZn having a long period structure was confirmed. Test pieces were cut from the extrusion goods. Their 0.2% proof stress, tensile strength and elongation were measured by conducting a tensile test on them at normal temperature. The results are shown in Table 1.

### [Referential Examples]

In Referential Examples, a metal structure of known magnesium alloys, that is, WE54-T6 material and AZ91 material was identified by X-ray diffraction and a transmission electron microscope, whereby the presence or absence of an intermetallic compound Mg₃Y₂Zn₃ and Mg₁₂YZn having a long period structure was confirmed. Test pieces were cut from the WE54-T6 material and AZ91 material, respectively. Their 0.2% proof stress, tensile strength and elongation were measured by conducting a tensile test on them at normal temperature. The results are shown in Table 1.

**[Table 1]**

| | Zn (at %) | Y(at%) | Zr(at%) | Zn/Y | Extrusion at (°C) | Intermetallic Compound Mg₃Y₂Zn₃ | Long-period phase Mg₁₂YZn | 0.2% Proof stress (MPa) stress (MPa) | Tensile strength (MPa) | Elongation (%) |
|---|---|---|---|---|---|---|---|---|---|---|
| Example 1 | 2 | 2 | - | 1 | 350 | ○ | ○ | 395 | 429 | 10.2 |
| Example 2 | 2 | 2 | - | 1 | 375 | ○ | ○ | 415 | 446 | 7.8 |
| Example 3 | 2 | 2 | 0.2 | 1 | 350 | ○ | ○ | 405 | 465 | 8.5 |
| Example 4 | 2 | 2 | 0.2 | 1 | 400 | ○ | ○ | 425 | 471 | 8.5 |
| Example 5 | 3 | 3 | - | 1 | 450 | ○ | ○ | 430 | 487 | 7.5 |
| Example 6 | 3 | 3.5 | - | 0.86 | 450 | ○ | ○ | 440 | 492 | 6 |
| Example 7 | 3.5 | 3 | - | 1.17 | 350 | ○ | ○ | 425 | 490 | 7.5 |
| Example 8 | 3.5 | 3.5 | - | 1 | 350 | ○ | ○ | 450 | 523 | 4.5 |
| Example 9 | 2.5 | 3 | - | 0.83 | 350 | ○ | ○ | 407 | 485 | 9 |
| Example 10 | 2 | 3 | - | 0.67 | 350 | ○ | ○ | 370 | 447 | 8.3 |
| Example 11 | 2.5 | 4 | - | 0.63 | 450 | ○ | ○ | 370 | 450 | 6 |
| Example 12 | 1.5 | 1.5 | - | 1 | 350 | ○ | ○ | 374 | 417 | 7.7 |
| Example 13 | 1 | 1 | - | 1 | 350 | ○ | ○ | 373 | 392 | 10.3 |
| Example 14 | 2 | 2 | - | 1.3 | 400 | ○ | ○ | 377 | 402 | 5.1 |
| Comparative Example 1 | 0.5 | 2 | - | 0.25 | 400 | × | ○ | 278 | 329 | 8.2 |
| Comparative Example 2 | 1 | 2 | - | 0.5 | 350 | × | ○ | 375 | 420 | 4 |
| Comparative Example 3 | 1 | 3 | - | 0.33 | 350 | × | ○ | 418 | 440 | 2 |
| Comparative Example 4 | 4 | 2 | - | 2 | 450 | ○ | × | 288 | 338 | 10.6 |
| Comparative Example 5 | 5 | 3 | - | 1.67 | 450 | ○ | × | 376 | 383 | 2.5 |
| Comparative Example 6 | 3 | 5 | - | 0.6 | 450 | × | ○ | 348 | 451 | 2.6 |
| Comparative Example 7 | 0.5 | 0.5 | - | 1 | 350 | × | ○ | 323 | 341 | 12 |
| Comparative Example 8 | 5 | 5 | - | 1 | 450 | ○ | ○ | 457 | 477 | 0.3 |
| Referential Example 1 | WE54-T6 material | | | - | -- | × | × | 172 | 250 | 2 |
| Referential Example 2 | AZ91 material | | | - | -- | × | × | 160 | 230 | 3 |

| | | | | | | | | | | |
|---|---|---|---|---|---|---|---|---|---|---|
| Intermetallic compound Mg₃Y₂Zn₃: O when it is contained, x when it is not contained Long-period phase Mg₁₂YZn: O when it is contained, x when it is not contained | | | | | | | | | | |

From Table 1, it is apparent that the magnesium alloys obtained in Examples 1 to 14 containing, based on the total alloy amount, from 1 to 4 atomic % of Zn and from 1 to 4.5 atomic % of Y at a Zn/Y composition ratio falling within a range of from 0.6 to 1.3, and containing both an intermetallic compound Mg₃Y₂Zn₃ and Mg₁₂YZn having a long period structure have both high strength and high ductility, because they are markedly superior to known WE54-T6 material and AZ91 material in each of strength (0.2% proof stress, tensile strength) and ductility (elongation).

Compared with the magnesium alloys obtained in Examples, those obtained in Comparative Examples 1 to 5 containing Zn and Y at a Zn/Y composition ratio outside the range of from 0.6 to 1.3 have only either one of the intermetallic compound Mg₃Y₂Zn₃ or Mg₁₂YZn having a long period structure, suggesting that they are not equipped sufficiently with either one or both of strength and ductility. It is apparent that the magnesium alloy obtained in Comparative Example 6 which contained Y in an amount exceeding the invention range of from 1 to 4.5 atomic % does not have the intermetallic compound Mg₃Y₂Zn₃ so that it does not have sufficient ductility. It is also apparent that the magnesium alloy obtained in Comparative Example 7 containing Zn in an amount less than the invention range of from 1 to 4 atomic % and Y in an amount less than the invention range of from 1 to 4.5 atomic % does not have the intermetallic compound Mg₃Y₂Zn₃ so that it does not have sufficient strength. It is also apparent that the magnesium alloy obtained in Comparative Example 8 containing Zn in an amount exceeding the invention range of from 1 to 4 atomic % and Y in an amount exceeding the invention range of from 1 to 4.5 atomic % contains both the intermetallic compound Mg₃Y₂Zn₃ and Mg₁₂YZn having a long period structure but it does not have sufficient ductility.

Provided are a magnesium alloy which is inexpensive, can be produced at a high yield, and has both high strength and high ductility; and a production process of the magnesium alloy. The magnesium alloy contains from 1 to 4 atomic % of Zn and from 1 to 4.5 atomic % of Y and optionally from 0.1 to 0.5 atomic % of Zr, at a Zn/Y composition ratio ranging from 0.6 to 1.3 as a remaining portion, Mg and inevitable impurities, and contains both an intermetallic compound Mg₃Y₂Zn₃, and Mg₁₂YZn having a long period structure. It may contain from 2 to 3.5 atomic % of Zn and from 2 to 4.5 atomic % of Y at a Zn/Y composition ratio falling within a range of from 0.8 to 1.2 and optionally from 0.1 to 0.5 atomic % of Zr. An alloy structure having both an intermetallic compound Mg₃Y₂Zn₃ and Mg₁₂YZn having a long period structure is available by casting an Mg alloy containing from 1 to 4 atomic % of Zn and from 1 to 4.5 atomic % of Y and optionally from 0,1 to 0,5 atomic % of Zr at a Zn/Y composition ratio ranging from 0.6 to 1.3 as a remaining portion, Mg and inevitable impurities, followed by plastic processing.

## Claims

1. A magnesium alloy, which comprises, based on a total amount, from 1 to 4 atomic % of Zn and from 1 to 4.5 atomic % of Y and optionally from 0.1 to 0.5 atomic % of Zr and as a remaining portion Mg and inevitable impurities , at a Zn/Y composition ratio falling within a range of from 0.6 to 1.3, and includes an intermetallic compound Mg₃Y₂Zn₃ and Mg₁₂YZn having a long period structure.

2. A magnesium alloy according to Claim 1, which comprises at least 3 atomic % of Zn and at least 3 atomic % of Y and optionally from 0.1 to 0.5 atomic % of Zr, each based on a total alloy amount, and as a remaining portion Mg and inevitable impurities.

3. A magnesium alloy according to Claim 1, which comprises from 2 to 3.5 atomic % of Zn and from 2 to 4.5 atomic % of Y and optionally from 0.1 to 0.5 atomic % of Zr, each based on a total alloy amount, at a Zn/Y composition ratio falling within a range of from 0.8 to 1.2.

4. A magnesium alloy according to Claim 3, which comprises at least 3 atomic % of Zn and at least 3 atomic % of Y and optionally from 0.1 to 0.5 atomic % of Zr, each based on a total alloy amount, and as a remaining portion Mg and inevitable impurities.

5. A production process of a magnesium alloy, which comprises casting a Mg alloy comprising from 1 to 4 atomic % of Zn and from 1 to 4.5 atomic % of Y, and optionally from 0.1 to 0.5 atomic % of Zr and as a remaining portion Mg and inevitable impurities, at a Zn/Y composition ratio falling within a range of from 0.6 to 1.3, using a cooling rate of 10 K/sec or less and a metal mould, graphite mould or sand mould; and plastic processing of the cast product obtained in the above described step into an alloy structure containing an intermetallic compound Mg₃Y₂Zn₃ and Mg₁₂YZn having a long period structure.

6. A production process of a magnesium alloy according to Claim 5, which comprises at least 3 atomic % of Zn and at least 3 atomic % of Y and optionally from 0.1 to 0.5 atomic % of Zr, each based on a total alloy amount, and as a remaining portion Mg and inevitable impurities.

7. A production process of a magnesium alloy according to Claim 5, which comprises from 2 to 3.5 atomic % of Zn and from 2 to 4.5 atomic % of Y and optionally from 0.1 to 0.5 atomic % of Zr, each based on a total alloy amount, at a Zn/Y composition ratio falling within a range of from 0.8 to 1.2.

8. A production process of a magnesium alloy according to Claim 7, wherein the magnesium alloy contains at least 3 atomic % of Zn and at least 3 atomic % of Y and optionally from 0.1 to 0.5 atomic % of Zr, each based on a total alloy amount and contains as a remaining portion Mg and inevitable impurities.

9. A production process of a magnesium alloy according to Claim 5, wherein the casting is performed at a cooling rate of 10 K/sec or less.

10. A production process of a magnesium alloy according to Claim 5, wherein the plastic processing is carried out by extrusion of the cast product.

## Patentansprüche

1. Magnesiumlegierung, die von 1 bis 4 Atom-% Zn und von 1 bis 4,5 Atom-% Y und gegebenenfalls von 0,1 bis 0,5 Atom-% Zr, bezogen auf die Gesamtmenge, und als verbleibenden Anteil Mg und unvermeidbare Verunreinigungen umfasst, wobei ein Zusammensetzungs-Verhältnis von Zn/Y in einen Bereich von 0,6 bis 1,3 fällt und die eine intermetallische Verbindung Mg₃Y₂Zn₃ und Mg₁₂YZn mit einer Langperioden-Struktur enthält.

2. Magnesiumlegierung nach Anspruch 1, die mindestens 3 Atom-% Zn und mindestens 3 Atom-% Y und gegebenenfalls von 0,1 bis 0,5 Atom-% Zr, jeweils bezogen auf die Gesamtmenge an Legierung, und als verbleibenden Anteil Mg und unvermeidbare Verunreinigungen umfasst.

3. Magnesiumlegierung gemäß Anspruch 1, die von 2 bis 3,5 Atom-% Zn und von 2 bis 4,5 Atom-% Y und gegebenenfalls von 0,1 bis 0,5 Atom-% Zr, jeweils bezogen auf die Gesamtmenge an Legierung, umfasst, wobei das Zusammensetzungsverhältnis von Zn/Y in einen Bereich von 0,8 bis 1,2 fällt.

4. Magnesiumlegierung gemäß Anspruch 3, die mindestens 3 Atom-% Zn und mindestens 3 Atom-% Y und gegebenenfalls von 0,1 bis 0,5 Atom-% Zr, jeweils bezogen auf die Gesamtmenge an Legierung, und als verbleibenden Anteil Mg und unvermeidbare Verunreinigungen umfasst.

5. Herstellungsverfahren einer Magnesiumlegierung, das das Gießen einer Magnesiumlegierung, die von 1 bis 4 Atom-% Zn und von 1 bis 4,5 Atom-% Y und gegebenenfalls von 0,1 bis 0,5 Atom-% Zr und als verbleibenden Anteil Mg und unvermeidbare Verunreinigungen umfasst, wobei das Zusammensetzungsverhältnis von Zn/Y in einen Bereich von 0,6 bis 1,3 fällt, mittels einer Abkühlrate von 10 K/s oder weniger und Verwenden einer Metallform, Graphitform oder Sandform, und das plastische Verarbeiten des Gießprodukts, das in dem oben beschriebenen Schritt erhalten wird, in eine Legierungsstruktur, die eine intermetallische Verbindung Mg₃Y₂Zn₃ und Mg₁₂YZn mit einer Langperioden-Struktur enthält, umfasst.

6. Herstellungsverfahren einer Magnesiumlegierung gemäß Anspruch 5, die mindestens 3 Atom-% Zn und mindestens 3 Atom-% Y und gegebenenfalls von 0,1 bis 0,5 Atom-% Zr, jeweils bezogen auf die Gesamtmenge an Legierung, und als verbleibenden Anteil Mg und unvermeidbare Verunreinigungen umfasst.

7. Herstellungsverfahren einer Magnesiumlegierung gemäß Anspruch 5, die von 2 bis 3,5 Atom-% Zn und von 2 bis 4,5 Atom-% Y und gegebenenfalls von 0,1 bis 0,5 Atom-% Zr, jeweils bezogen auf die Gesamtmenge an Legierung, umfasst, wobei ein Zusammensetzungsverhältnis von Zn/Y in einen Bereich von 0,8 bis 1,2 fällt.

8. Herstellungsverfahren einer Magnesiumlegierung gemäß Anspruch 7, wobei die Magnesiumlegierung mindestens 3 Atom-% Zn und mindestens 3 Atom-% Y und gegebenenfalls von 0,1 bis 0,5 Atom-% Zr, jeweils bezogen auf die Gesamtmenge an Legierung, enthält und als verbleibenden Anteil Mg und unvermeidbare Verunreinigungen enthält.

9. Herstellungsverfahren einer Magnesiumlegierung gemäß Anspruch 5, wobei das Gießen bei einer Abkühlrate von 10 K/s oder weniger durchgeführt wird.

10. Herstellungsverfahren einer Magnesiumlegierung gemäß Anspruch 5, wobei das plastische Verarbeiten durch Extrusion des Gießprodukts durchgeführt wird.

## Revendications

1. Alliage de magnésium qui comprend, sur la base d'une quantité totale, de 1 à 4 % atomique de Zn et de 1 à 4,5 % atomique de Y et éventuellement de 0,1 à 0,5 % atomique de Zr, et en tant que partie restante, du Mg et des impuretés inévitables, à un rapport de composition Zn/Y s'inscrivant dans la gamme de 0,6 à 1,3, et comprend un composé intermétallique Mg₃Y₂Zn₃ et Mg₁₂YZn ayant une structure à longue période.

2. Alliage de magnésium selon la Revendication 1, qui comprend au moins 3 % atomique de Zn et au moins 3 % atomique de Y et éventuellement de 0,1 à 0,5 % atomique de Zr, chacun sur la base d'une quantité d'alliage totale, et en tant que partie restante, du Mg et des impuretés inévitables.

3. Alliage de magnésium selon la Revendication 1, qui comprend de 2 à 3,5 % atomique de Zn et de 2 à 4,5 % atomique de Y et éventuellement de 0,1 à 0,5 % atomique de Zr, chacun sur la base d'une quantité d'alliage totale, à un rapport de composition Zn/Y s'inscrivant dans la gamme de 0,8 à 1,2.

4. Alliage de magnésium selon la Revendication 3, qui comprend au moins 3 % atomique de Zn et au moins 3 % atomique de Y et éventuellement de 0,1 à 0,5 % atomique de Zr, chacun sur la base d'une quantité d'alliage totale, et en tant que partie restante, du Mg et des impuretés inévitables.

5. Procédé de préparation d'un alliage de magnésium, qui comprend la coulée d'un alliage Mg comprenant de 1 à 4 % atomique de Zn et de 1 à 4,5 % atomique de Y, et éventuellement de 0,1 à 0,5 % atomique de Zr, et en tant que partie restante, du Mg et des impuretés inévitables, à un rapport de composition Zn/Y s'inscrivant dans la gamme de 0,6 à 1,3, utilisant une vitesse de refroidissement de 10 K/sec ou moins et un moule en métal, un moule en graphite ou un moule en sable ; et la transformation plastique du produit coulé obtenu au cours de l'étape décrite ci-dessus en une structure d'alliage contenant un composé intermétallique Mg₃Y₂Zn₃ et Mg₁₂YZn ayant une structure à longue période.

6. Procédé de préparation d'un alliage de magnésium selon la Revendication 5, qui comprend au moins 3 % atomique de Zn et au moins 3 % atomique de Y, et éventuellement de 0,1 à 0,5 % atomique de Zr, chacun sur la base d'une quantité d'alliage totale, et en tant que partie restante, du Mg et des impuretés inévitables.

7. Procédé de préparation d'un alliage de magnésium selon la Revendication 5, qui comprend de 2 à 3,5 % atomique de Zn et de 2 à 4,5 % atomique de Y, et éventuellement de 0,1 à 0,5 % atomique de Zr, chacun sur la base d'une quantité d'alliage totale, à un rapport de composition Zn/Y s'inscrivant dans la plage de 0,8 à 1,2.

8. Procédé de préparation d'un alliage de magnésium selon la Revendication 7, dans lequel l'alliage de magnésium contient au moins 3 % atomique de Zn et au moins 3 % atomique de Y, et éventuellement de 0,1 à 0,5 % atomique de Zr, chacun sur la base d'une quantité d'alliage totale, et contient, en tant que partie restante, du Mg et des impuretés inévitables.

9. Procédé de préparation d'un alliage de magnésium selon la Revendication 5, dans lequel la coulée est effectuée à une vitesse de refroidissement de 10 K/sec ou moins.

10. Procédé de préparation d'un alliage de magnésium selon la Revendication 5, dans lequel la transformation plastique est effectuée par extrusion du produit coulé.
